

## UNITED STATES PATENT OFFICE

2,336,260

DIFFUSION OF SENSITIZING DYES IN  
PHOTOGRAPHIC EMULSIONS

Edward B. Knott, Wealdstone, Harrow, England,  
assignor to Eastman Kodak Company, Rochester, N. Y., a corporation of New Jersey

No Drawing. Application May 1, 1941, Serial No.  
391,375. In Great Britain June 6, 1940

15 Claims. (Cl. 95—7)

This invention relates to the diffusion of sensitising dyes in photographic emulsions and more particularly to the retardation of such diffusion.

For certain purposes in photography, there are required sensitive papers, films, plates and similar materials comprising two or more emulsions which respond in different ways to differently colored light. Thus, one of the emulsions may be insensitive to light of a color to which a second emulsion may be sensitive. In the production of these sensitive materials, the emulsions are sometimes mixed before application to the support, while in other instances, the emulsions are applied successively in layers to the support. For example, it is common practice in the production of sensitive materials for use in color photography to apply successively to the support layers emulsions sensitive to different regions of the spectrum. In certain instances, in color photographic elements, two or more emulsions are mixed together in one layer.

As a further example of the use of sensitive materials comprising two or more emulsions which respond in different ways to differently colored light, may be mentioned printing papers which are capable of giving a result of high or low contrast, depending upon the color of the light used in printing. Such papers can be produced by applying to a paper support a mixture of two emulsions, one of which gives an image of high contrast and can be printed by using light of one color, and the second gives an image of low contrast and can be printed by using a light of different color. Instead of a mixture of two emulsions, the emulsions can be applied successively to the paper support. The emulsion used in such printing papers, or in the aforementioned color photographic materials, may be all of one type, say silver chloride or silver bromide, or the emulsions may be of different types.

Whether the emulsions are of the same or of different types, the different sensitivities of the emulsions to differently colored light can be controlled by means of sensitizing dyes. Thus, one emulsion may be prepared free from sensitizing dye and hence sensitive to blue light but not to light of longer wavelengths, while the other emulsion may contain a dye which sensitizes the emulsion to yellow light, in which case the second emulsion will be sensitive both to yellow and to blue light, since the emulsion possesses a natural sensitivity to blue. Alternatively the two emulsions may contain different sensitizing dyes, so that each emulsion is dye-sensitized for a different spectral region.

Numerous sensitizing dyes which may be employed are known, including among others, sensitizing dyes from the cyanine, the hemicyanine, the merocyanine, the oxonol and the hemioxonal dye classes. In practice, however, the sensitizing dye or dyes adsorbed on the grains of one emulsion have a greater or lesser tendency to wander or diffuse to the grains of another emulsion where the dye is not desired. When the 5 grains of the two emulsions are adjacent, that is sufficiently close, for example when the emulsions are mixed or coated in immediate contact one on the other; such diffusion occurs almost solely during the time in which the emulsions 10 are adjacent in the wet condition. If such diffusion occurs the initial difference in sensitivity between the emulsions is, of course, reduced, and may even be lost practically entirely. Even where the emulsions are applied in consecutive 15 layers, the tendency of certain dyes to wander from one layer to another is very marked. Only a relatively few of the well-known powerful sensitizing dyes have low enough resistance to wander to be useful in the production of photographic materials of the kind described above.

To reduce this undesirable tendency to wander, it has been proposed to introduce into the 20 molecules of the sensitizing dyes, long chain organic groups. Dye molecules containing such chains show a lesser tendency to diffuse, but such dyes also show a greater or lesser decrease in 25 sensitizing power, depending upon the point of attachment of the long-chain organic group. At best, such a method of retarding diffusion is at 30 the expense of sensitizing power. It has also been proposed to retard wandering of quaternary 35 salt types of sensitizing dyes in photographic emulsions by incorporating perchlorates, such as sodium perchlorate, in the emulsions containing 40 the dyes. However, this method leaves much to be desired, and in the case of non-quaternary 45 salt types of dyes, such as merocyanine dyes, the method is of no utility whatsoever.

It is accordingly an object of my invention to 45 provide a process for retarding such diffusion of sensitizing dyes. Another object is to provide emulsions containing sensitizing dyes which are retarded from diffusion. Other objects will become apparent hereinafter.

50 I have found that the tendency for sensitizing dyes of all types, and particularly dyes of the above-mentioned types, to wander or diffuse from the grains of one photographic silver halide emulsion, to the grains of an adjacent silver halide emulsion, can be substantially reduced by 55

dispersing in the emulsion a substantially water-insoluble metal compound preferably before bringing the emulsions into contact and also preferably after the sensitising dye. I have found that substantially water-insoluble metal oxides, metal hydroxides, metal oxysalts and metal hydroxysalts are advantageously employed.

In practicing my invention, to obtain the best results the following conditions should be observed. It is important that such water-insoluble metal compound should be incorporated in the emulsion before it is brought into contact

In the case of each water-insoluble compound tested some of the mixed emulsion was coated immediately after the mixing and then dried while some was coated after being kept in the wet condition at 35° C. Some compounds were found to prevent wandering even under the latter rather severe test conditions while others were satisfactory for immediate coating but showed a little wandering after the two hours keeping in the wet condition. The dye-wandering was observed by means of wedge spectrograms. The following table shows the effects obtained:

Table

| Water-insoluble metal compound                         | Effect on wandering            | Effect on speed                                                                                                      | pH of gelatin suspension |
|--------------------------------------------------------|--------------------------------|----------------------------------------------------------------------------------------------------------------------|--------------------------|
| ZnO                                                    | Stops wandering                | No change                                                                                                            | 6.0                      |
| TiO <sub>2</sub>                                       | Reduces wandering              | Slight speed loss in dye-sensitised emulsion                                                                         | 5.4                      |
| Al <sub>2</sub> O <sub>3</sub>                         | do                             | No change                                                                                                            | 6.0                      |
| ZrO <sub>2</sub>                                       | do                             | No change (loss in gamma)                                                                                            | 6.0                      |
| Sb <sub>2</sub> O <sub>3</sub>                         | do                             | do                                                                                                                   | 6.0                      |
| Bi <sub>2</sub> O <sub>3</sub>                         | do                             | Increase of speed of dye-sensitised emulsion                                                                         | 6.0                      |
| La <sub>2</sub> O <sub>3</sub>                         | Almost stops wandering         | Lowers gamma                                                                                                         | 8.0                      |
| SnO <sub>2</sub>                                       | Reduces wandering              | do                                                                                                                   | 5.6                      |
| Y <sub>2</sub> O <sub>3</sub>                          | do                             | do                                                                                                                   | 4.5                      |
| MgO                                                    | Almost stops wandering         | Great increase in speed of dye-sensitised emulsion; slight increase in speed of unsensitised emulsion                | 9.0                      |
| CaO                                                    | do                             | do                                                                                                                   | 9.0                      |
| Mg(OH) <sub>2</sub>                                    | do                             | do                                                                                                                   | 9.0                      |
| Ca(OH) <sub>2</sub>                                    | do                             | Great increase in speed of dye-sensitised emulsion; slight increase in speed of unsensitised emulsion (tends to fog) | 9.0                      |
| BiOCl                                                  | Reduces wandering considerably | No change                                                                                                            | 4.8                      |
| $\text{Al}_2(\text{OH})_2\left(\text{OCCH}_3\right)_2$ | Reduces wandering              | Lowers gamma of unsensitised emulsion                                                                                | 4.0                      |
| BaSO <sub>4</sub>                                      | do                             | No change                                                                                                            | 6.0                      |

with another emulsion. Where it is desired that two adjacent emulsions should both be sensitized but with different dyes then each emulsion should be sensitized and have incorporated in it a water insoluble metal compound before the two emulsions are brought into contact. The water-insoluble metal compound can be added to the emulsion in the form of a finely divided powder or precipitate. More advantageously however, the water-insoluble metal compound is first emulsified in a 5 per cent solution of gelatin in water, the emulsification being followed by centrifuging to remove all but the finest grains of water-insoluble compound. A suspension of the water-insoluble metal compound can also be formed by precipitation of the water-insoluble metal compound in a gelatin solution. However prepared, such a gelatin suspension of the water-insoluble metal compound provides an advantageous form in which to add the water-insoluble metal compound to the emulsion. The water-insoluble metal compound should, of course, be thoroughly incorporated throughout the emulsion.

The concentration of the water-insoluble metal compound which is most advantageously employed will depend, of course, upon the silver halide emulsion employed and upon the sensitising dye employed. Ordinarily, however, from about 10 to about 150 grams of water-insoluble metal compound per gram-mole of silver halide in the emulsion will suffice to retard wandering of the sensitising dyes to an adjacent emulsion.

The following procedure was found satisfactory to determine the effect of the various water-insoluble metal compounds. To a hard silver chloride emulsion was added a green sensitising dye and the emulsion was held at 35° C. for 30 minutes. A gelatin suspension of the water-insoluble compound was then added, and this was followed by a blue sensitive soft bromide emulsion.

35 Zinc oxide is the most efficacious of the materials listed in the above table. After two hours keeping in the wet condition at 35° C. of the mixed emulsion containing zinc oxide, there was no wandering of the sensitising dyes. The lower the colour sensitivity of the emulsion compared with the natural blue sensitivity of the other emulsion, the greater is the necessity to use water insoluble compounds which are highly efficacious, using if necessary also a water insoluble resin to improve the effect still further. As shown in the copending application of Edward P. Davey, Serial No. 387,437, filed April 8, 1941, incorporation of water-insoluble resins in photographic gelatino-silver-halide emulsions not earlier than the sensitising dyes, serves to retard diffusion of the sensitising dyes. Thus, from about 10 to about 35 grams of resins, such as whole shellac, soft shellac, hard shellac, hydrolysed shellac, colophony, dammar, sandarach, mastic or glyptals, per gram-mole of silver halide in the emulsion serves to retard diffusion of sensitising dyes. I have now found with a mixture of my water-insoluble metal compounds and substantially water-insoluble resins, e. g., those set forth above, that the components of the mixture co-operate to retard diffusion of sensitising dyes in a highly efficacious manner.

60 The following example will serve to illustrate the practice of my invention.

#### Example 1

Two gelatino-silver-halide emulsions were selected, the one being a hard silver chloride developing-out emulsion and the other being a soft silver bromide developing-out emulsion. The silver ratio of the two emulsions was one to one. The pH of each emulsion was adjusted to 7.0. The chloride emulsion was sensitised with 5-[ $(3$ -ethyl-2(3) - benzoxazolylidene) - ethylidene]-3-ethyl-1-phenyl-2-thiohydantoin. The sensitised

emulsion was allowed to stand at 35° C. for 30 minutes. To this sensitised emulsion, which contained the equivalent of 200 grams of silver nitrate, were then added a gelatin suspension of 20 grams of magnesium oxide followed by 30 grams of soft shellac resin contained in ethyl alcoholic solution (5 per cent by weight of resin). The resulting mixture was kept at 35° C. for a period of time, depending upon the final chloride speed desired (say for 90 minutes). To the soft bromide emulsion were added the same amounts of magnesium oxide and resin. The two emulsions were then mixed. The mixed emulsion can be coated immediately or after standing, say for one hour.

Apart from the fact that the oxides of magnesium, calcium and lanthanum retard sensitising dye diffusion, these oxides cause a substantial rise in the speed of the dye-sensitised emulsion. This speed rise is dependent upon two factors, (1) the ratio of oxide to silver in the emulsion and (2) the time of keeping of the dye-sensitised emulsion in the liquid state with the oxide, before coating. There is a gradual speed rise over a period of several hours until the emulsion runs into stain. The hydroxides of calcium, magnesium and lanthanum function in the same way, and probably the effect of the oxides is due to their becoming hydrated to the corresponding hydroxides. While these oxides and hydroxides are substantially water-insoluble, they are slightly soluble in water and, therefore, give the emulsions a high pH. The speed increase due to this high pH, however, is very slight.

In general from about 10 to about 20 grams of the oxides or hydroxides of calcium, magnesium or lanthanum per gram-mole of silver halide will substantially retard diffusion without greatly affecting speed, whereas from about 75 to about 125 grams per gram-mole of silver halide will not only substantially retard diffusion of the sensitising dyes, but will considerably increase the speed of the dye-sensitised emulsion.

With the oxides and hydroxides of calcium, magnesium and lanthanum, the sensitising dyes should be selected with especial care, since these substances tend to decompose some sensitising dyes upon standing with them.

Since the refractive indices of magnesium hydroxide and certain glyptal resins are almost the same as that of gelatin, clear films can be obtained when employing a combination of these two substances.

For best results, I have found that the hard chloride emulsions employed should contain an excess of soluble chlorides.

In accordance with a further embodiment of my invention, I incorporate in the emulsions along with the water-insoluble metal compound, a water soluble metal salt of a resin. The water-insoluble metal compound and the water-soluble metal salt of the resin co-operate to retard diffusion of the sensitising dyes in an efficacious manner. Water soluble metal salts of resins which are advantageously employed are the alkali metal or ammonium salts of resins, such as whole lac, hard lac, soft lac, hydrolysed lac, colophony, dammar, sandarach, mastic and glyptals.

In accordance with a still further embodiment of my invention, I retard diffusion of sensitising dyes from the grains of one photographic gelatino-silver-halide emulsion to the grains of another adjacent emulsion by incorporating in

the emulsion substantially water-insoluble metal salts of resins preferably before bringing the emulsions into contact, and preferably after the sensitising dye. This is advantageously accomplished by incorporating in the emulsion a water-soluble metal salt or hydroxide and a water-soluble metal salt of a resin, the water-soluble metal salt being one which contains a cation which reacts with the water-soluble metal salt of a resin to give a substantial water-insoluble metal salt of a resin.

The following list gives some of the water-soluble metal salts and water-soluble metal salts of resins which can be employed effectively:

15

| Water soluble metal salts or hydroxides | Water soluble metal salts or resins                             |
|-----------------------------------------|-----------------------------------------------------------------|
| Any water soluble salt or hydroxide of— | Ammonium or alkali metal (e. g., potassium or sodium) salts of— |
| Aluminum                                | Whole lac                                                       |
| Barium                                  | Hard lac                                                        |
| Cadmium                                 | Soft lac                                                        |
| Calcium                                 | Hydrolysed lac                                                  |
| Cerium                                  | Colophony                                                       |
| Cobalt                                  | Dammar                                                          |
| Copper                                  | Sandarach                                                       |
| Magnesium                               | Mastic                                                          |
| Manganese                               | Glyptals                                                        |
| Strontium                               |                                                                 |
| Thorium                                 |                                                                 |
| Zinc                                    |                                                                 |

30

In carrying out my invention according to the preferred embodiment, I first adjust the pH of the gelatino-silver halide emulsion to at least 7. To the sensitised emulsion I then add a one per cent aqueous solution of the water-soluble metal salt or hydroxide followed by a 5 per cent aqueous solution of the water soluble metal salt of a resin. Sufficient of the two solutions are incorporated to give from about 10 to about 35 grams of water-insoluble metal salt of a resin per gram-mole of silver halide in the emulsion.

The following example will serve to illustrate the practice of my invention.

A hard gelatino-silver-chloride developing-out emulsion sensitised with 5-[3-ethyl-2(3)-benzoxazolylidene)-ethylenel-3-ethyl-1-phenyl - 2-thiohydantoin containing the equivalent of 200 grams of silver nitrate was adjusted to a pH of at least 7. To the resulting emulsion were added a 1 per cent aqueous solution of 5 grams of cadmium nitrate. The cadmium nitrate was thoroughly incorporated in the emulsion, and a slow stream of a 5 per cent aqueous solution of 30 grams of the sodium salt of colophony were added. After a wait of 15 minutes, a soft gelatino-silver-bromide developing-out emulsion was mixed with the chloride emulsion. Such a mixed emulsion can be kept at 35° C. for some hours without dye wandering into the grains of the other emulsion. It is preferable to incorporate also in the soft bromide emulsion a water-insoluble metal salt of a resin in the same manner as described for the hard chloride emulsion.

Instead of cadmium nitrate, 5 grams of zinc chloride or 5 grams of cobalt ammonium sulfate were found to give good results. Likewise, the sodium salt of colophony was replaced with the sodium salt of soft lac resin in connection with cadmium nitrate, zinc chloride and cobalt ammonium sulfate, and efficacious retardation of diffusion of the sensitising dye was obtained.

In accordance with any of the embodiments of my invention, diffusion of sensitising dyes from the cyanine class, the merocyanine class (see U. S. Patent 2,078,233, dated April 27, 1937),

the hemicyanine class (see U. S. Patent 2,166,736, dated July 18, 1939), the hemioxonal class (see U. S. Patent 2,216,441, dated October 1, 1940), and the oxonal class (see the copending application of L. G. S. Brooker and G. H. Keyes, Serial No. 270,916, filed April 29, 1939) can be retarded.

What I claim and desire to be secured by Letters Patent of the United States is:

1. A photographic element comprising at least two photographic silver halide emulsions positioned with the grains of one emulsion adjacent to the grains of another emulsion, at least one of said emulsions being sensitized with a sensitizing dye, at least the emulsions sensitized with a sensitizing dye containing a substantially water-insoluble metal compound selected from the group consisting of metal oxides, metal hydroxides, metal oxsalts, metal hydroxysalts and metal salts of resins, to retard diffusion of the sensitizing dye, said metal compound having been incorporated in the emulsion after the sensitizing dye.

2. A photographic element comprising at least two photographic gelatino silver halide emulsions positioned with the grains of one emulsion adjacent to the grains of another emulsion, at least one of said emulsions being sensitized with a sensitizing dye, at least the emulsions sensitized with a sensitizing dye containing a substantially water-insoluble metal compound selected from the group consisting of metal oxides, metal hydroxides, metal oxsalts, metal hydroxysalts and metal salts of resins, to retard diffusion of the sensitizing dye, said metal compound having been incorporated in the emulsion after the sensitizing dye.

3. A photographic element comprising at least two photographic gelatino silver halide emulsions positioned with the grains of one emulsion adjacent to the grains of another emulsion, at least one of said emulsions being sensitized with a sensitizing dye, at least the emulsions sensitized with a sensitizing dye containing a substantially water-insoluble metal compound selected from the group consisting of calcium, magnesium, lanthanum and zinc oxides and hydroxides, to retard diffusion of the sensitizing dye, said metal compound having been incorporated in the emulsion after the sensitizing dye.

4. A photographic element comprising at least two photographic gelatino silver halide emulsions positioned with the grains of one emulsion adjacent to the grains of another emulsion, at least one of said emulsions being sensitized with a sensitizing dye, at least the emulsions sensitized with a sensitizing dye containing a substantially water-insoluble metal compound selected from the group consisting of magnesium hydroxide and magnesium oxide, to retard diffusion of the sensitizing dye, said metal compound having been incorporated in the emulsion after the sensitizing dye.

5. A photographic element comprising at least two photographic gelatino silver halide emulsions positioned with the grains of one emulsion adjacent to the grains of another emulsion, at least one of said emulsions being sensitized with a sensitizing dye, at least the emulsions sensitized with a sensitizing dye containing a substantially water-insoluble metal compound selected from the group consisting of zinc hydroxide and zinc oxide, to retard diffusion of the sensitizing dye,

said metal compound having been incorporated in the emulsion after the sensitizing dye.

6. A photographic element comprising at least two photographic gelatino silver halide emulsions positioned with the grains of one emulsion adjacent to the grains of another emulsion, at least one of said emulsions being sensitized with a sensitizing dye, at least the emulsions sensitized with a sensitizing dye containing a substantially water-insoluble metal compound selected from the group consisting of lanthanum hydroxide and lanthanum oxide, to retard diffusion of the sensitizing dye, said metal compound having been incorporated in the emulsion after the sensitizing dye.

7. A photographic element comprising at least two photographic gelatino silver halide emulsions positioned with the grains of one emulsion adjacent to the grains of another emulsion, at least one of said emulsions being sensitized with a sensitizing dye, at least the emulsions sensitized with a sensitizing dye containing, in a concentration of from about 10 grams to about 150 grams per gram-mole of silver halide in the emulsions, a substantially water-insoluble metal compound selected from the group consisting of metal oxides, metal hydroxides, metal oxsalts, metal hydroxysalts and metal salts of resins, to retard diffusion of the sensitizing dye, said metal compound having been incorporated in the emulsion after the sensitizing dye.

8. A photographic element comprising at least two photographic gelatino silver halide emulsions positioned with the grains of one emulsion adjacent to the grains of another emulsion, at least one of said emulsions being sensitized with a sensitizing dye, at least the emulsions sensitized with a sensitizing dye containing a substantially water-insoluble metal compound selected from the group consisting of metal oxides, metal hydroxides, metal oxsalts, metal hydroxysalts and metal salts of resins, and containing a substantially water-insoluble resin, to retard diffusion of the sensitizing dye, said metal compound and said resin having been incorporated in the emulsion after the sensitizing dye.

9. A photographic element comprising at least two photographic gelatino silver halide emulsions positioned with the grains of one emulsion adjacent to the grains of another emulsion, at least one of said emulsions being sensitized with a sensitizing dye, at least the emulsions sensitized with a sensitizing dye containing a substantially water-insoluble metal compound selected from the group consisting of calcium, magnesium, lanthanum and zinc oxides and hydroxides, and containing a substantially water-insoluble resin, to retard diffusion of the sensitizing dye, said metal compound and said resin having been incorporated in the emulsion after the sensitizing dye.

10. A photographic element comprising at least two photographic gelatino silver halide emulsions positioned with the grains of one emulsion adjacent to the grains of another emulsion, at least one of said emulsions being sensitized with a sensitizing dye, at least the emulsions sensitized with a sensitizing dye containing magnesium oxide and soft lac resin, to retard diffusion of the sensitizing dye, said magnesium oxide and soft lac resin having been incorporated in the emulsion after the sensitizing dye.

11. A photographic element comprising at least two photographic gelatino silver halide emulsions positioned with the grains of one emulsion

adjacent to the grains of another emulsion, one of said emulsions being sensitized with a merocyanine dye and containing magnesium oxide and soft lac resin to retard diffusion of the sensitizing dye, said magnesium oxide and soft lac resin having been incorporated in the emulsion after the merocyanine dye.

12. A photographic element comprising a contrasty gelatino silver chloride emulsion sensitized to the green with a sensitizing dye, and a soft gelatino silver bromide emulsion positioned with its grains adjacent to the grains of the contrasty chloride emulsion, both the chloride and the bromide emulsion containing magnesium oxide and soft lac resin to retard diffusion of the sensitizing dye, said magnesium oxide and soft lac resin having been incorporated in the emulsion after the sensitizing dye.

13. A process for preparing a photographic element comprising incorporating in at least one of two photographic silver halide emulsions, prior to bringing the emulsions into contact, a sensitizing dye, and after incorporation of the sensitizing dye in the emulsion, incorporating in at least the dye-sensitized emulsion a substantially water-insoluble metal compound selected from the group consisting of metal oxides, metal hydroxides, metal oxysalts, metal hydroxysalts and metal salts of resins, and then bringing the two emulsions into contact.

resins, and then bringing the two emulsions into contact.

14. A process for preparing a photographic element comprising incorporating in at least one of two photographic gelatino silver halide emulsions, prior to bringing the emulsions into contact, a sensitizing dye, and after incorporation of the sensitizing dye in the emulsion, incorporating in at least the dye-sensitized emulsion a substantially water-insoluble metal compound selected from the group consisting of metal oxides, metal hydroxides, metal oxysalts, metal hydroxysalts and metal salts of resins, and then bringing the two emulsions into contact.

15. A process for preparing a photographic element comprising incorporating in at least one of two photographic gelatino silver halide emulsions, prior to bringing the emulsions into contact, a sensitizing dye, and after incorporation of the sensitizing dye in the emulsion, incorporating in at least the dye-sensitized emulsion a substantially water-insoluble metal compound selected from the group consisting of metal oxides, metal hydroxides, metal oxysalts, metal hydroxysalts and metal salts of resins and then bringing the emulsions into contact.

EDWARD B. KNOTT.